

Apr. 17, 1923.

1,452,364

W. T. DAVIS

METHOD OF PURIFYING MOLTEN METAL

Filed May 20, 1921



INVENTOR.

Walter T. Davis,  
of Bakewell, Barnes & Parmelle,  
his atty.

## UNITED STATES PATENT OFFICE.

WALTER T. DAVIS, OF WHEELING, WEST VIRGINIA, ASSIGNOR TO WHEELING STAMPING COMPANY, OF WHEELING, WEST VIRGINIA, A CORPORATION OF WEST VIRGINIA.

## METHOD OF PURIFYING MOLTEN METAL.

Application filed May 20, 1921. Serial No. 471,104.

*To all whom it may concern:*

Be it known that I, WALTER T. DAVIS, a resident of Wheeling, Ohio County, West Virginia, have invented a new and useful 5 Improvement in Methods of Purifying Molten Metal, of which the following is a full, clear, and exact description, reference being had to the accompanying drawing, forming part of this specification, in which the figure 10 is a vertical section of one form of apparatus for carrying out my invention.

My invention has relation to the purification of molten metal, such as molten tin, or/and lead.

15 It is highly desirable in using molten metals of the character above stated that they shall be freed as far as possible from dust and dirt which are usually present to a large degree therein, these metals being ordinarily melted within open tanks or vessels.

I have discovered that this purification can be accomplished in a very thorough and effective manner by causing the discharge of air at the bottom portion of the tank containing the molten metal and causing such air to bubble upwardly through the metal. The escaping bubbles of air serve to catch and carry with them to the surface of the metal a very large part of the contained 25 dust and dirt. When carried in this manner to the surface of the molten bath of metal, the dirt mingles with the dross or scum formed by oxidation, and can be readily removed by skimming.

30 35 My invention can be carried out in various ways, one of which I have illustrated in the accompanying drawing. In this draw-

ing, the numeral 2 designates any suitable vessel or tank containing the body of molten metal to be purified. 3 designates an air 40 pipe connected with a source of air under pressure, and it is extended into the tank and along the bottom portion thereof. This pipe is provided with a plurality of small perforations 4, through which air may escape 45 and pass upwardly through the molten metal.

Any desired number of these pipes may be arranged in the tank in any suitable manner, the best results being obtained when the pipe arrangement is such that air will be caused to escape and pass upwardly through 50 the major portion of the volume of the bath.

55 My invention forms a very simple and efficient method for the purpose described and by the use of which the molten metal may be very largely freed from contained dirt.

I claim:

1. The herein described method of purifying molten tin or/and lead metal, which consists in liberating air at the lower portion of the mass of metal to be purified, and causing said air to pass upwardly through the body of metal, substantially as described.

2. The herein described method of purifying molten tin or/and lead metal, which consists in releasing air under pressure in a plurality of small streams at the lower portion of the body of metal to be purified, and allowing the liberated air to pass upwardly through the body of metal, substantially as described.

In testimony whereof, I have hereunto set my hand.

WALTER T. DAVIS.